

# UNITED STATES PATENT OFFICE.

FERDINAND STERNBERG, OF NEW YORK, N. Y., ASSIGNOR OF ONE-HALF TO JOHN FOLCZ, OF NEW YORK, N. Y.

## PAINT COMPOSITION.

1,110,358.

Specification of Letters Patent. Patented Sept. 15, 1914.

No Drawing.

Application filed December 30, 1913. Serial No. 809,479.

To all whom it may concern:

Be it known that I, FERDINAND STERNBERG, a subject of the Emperor of Germany, and resident of the city of New York, in the county of New York and State of New York, have invented certain new and useful Improvements in a Paint Composition, of which the following is a specification.

This invention relates to a paint composition, and more especially to a composition for green paint adapted for use upon metal articles.

An object of the invention is to provide a paint for use upon metal articles and especially automobile bodies which will produce a high degree of gloss and luster of a character that will not grow dull but will remain free from dust.

A still further object is to provide a brilliant green paint having the appearance of reflecting various metallic colors and upon being applied with a painter's brush in the usual manner, will produce a glistening sparkling finish with a green background having a twinkling reflecting effect.

My compound is prepared in the form of a paint powder and it consists of the following ingredients combined in substantially the proportions hereinafter specified.

|    |                          |           |
|----|--------------------------|-----------|
| 30 | Green ultramarine        | 100 parts |
|    | Verdigris                | 25 parts  |
|    | Finely pulverized copper | 15 parts  |
|    | Indigo blue              | 25 parts  |
| 35 | Prepared violet anilin   | 5 parts   |

All of the above ingredients are finely powdered and then thoroughly mixed together, and in preparing for use, a further mixing of said powdered ingredients is had with varnish and japan as a drier.

When employed upon small articles, the

articles so coated may be dried or baked in an oven.

This paint may be employed upon wood if desired although especially adapted for 45 coating metal.

While I am aware that one or more of the above ingredients such as anilin, has heretofore been employed in a paint composition, I am not aware that the combination of all 50 of my ingredients has ever been so employed nor that the relative proportions named have ever been used, and I therefore confine myself to the ingredients employed and the purpose stated. Commingling of all 55 of said ingredients unitedly into a single composition and most perfectly in the exact proportions named, produces an untarnishing paint coating for metal superior to that which is obtained by the separate use or 60 substitution for any of the ingredients now employed. It will also be apparent that a different color may be produced by changing the color of the predominating element.

Having thus described my invention, what 65 I claim as new and desire to secure by Letters Patent of the United States is:—

1. A paint composition containing green ultramarine, verdigris, pulverized copper, 70 indigo blue, and violet anilin in substantially the proportions set forth.

2. A paint composition containing green ultramarine 100 parts, verdigris 25 parts, finely powdered copper 15 parts, indigo blue 75 25 parts, and prepared violet anilin 5 parts.

Signed at the city of New York, in the county of New York, and State of New York, this 26th day of December, A. D. 1913.

FERDINAND STERNBERG.

Witnesses:

M. SCHNITZER,  
E. ELKINSON.